

(No Model.)

M. R. CONLEY.  
PROCESS OF MAKING IRON OR STEEL.

No. 534,857.

Patented Feb. 26, 1895.



FIG. 2.



WITNESSES:

George Baumann  
S. C. Connor

INVENTOR  
Michael R. Conley

BY  
Howson and Howson  
his ATTORNEYS.

# UNITED STATES PATENT OFFICE.

MICHAEL R. CONLEY, OF BROOKLYN, ASSIGNOR TO WILLIAM BELL, OF NEW YORK, N. Y.

## PROCESS OF MAKING IRON OR STEEL.

SPECIFICATION forming part of Letters Patent No. 534,857, dated February 26, 1895.

Application filed April 17, 1894. Serial No. 507,868. (No specimens.)

To all whom it may concern:

Be it known that I, MICHAEL R. CONLEY, a citizen of the United States, and a resident of Brooklyn, Kings county, New York, have 5 invented an Improved Process of Making Iron or Steel, of which the following is a specification.

My invention consists of an improved process of making iron or steel from fine, pulverized ore and scrap.

To carry my method into effect I prefer to use a construction of furnace which is an improvement upon that for which I obtained Letters Patent No. 477,623, dated June 21, 15 1892.

In the accompanying drawings, Figure 1 is a longitudinal section of my improved furnace, and Fig. 2 is a transverse section on the line 1—2, Fig. 1.

It will facilitate the explanation and understanding of my process, if I first describe the construction of furnace employed for carrying it into effect.

As in my former furnace I have a central 25 open hearth combined with reverberatory furnaces and retorts, so located in flues at opposite sides of the open hearth as that the said retorts may be heated by the waste heat or gases passing from the open hearth, and this 30 without interfering with the reversing principle of the reverberatory open hearth furnace, and without using any other regenerators than those needed for the melting hearth.

The furnace may be constructed in general after the manner of the Siemens reverberatory steel melting furnace with its gas and air regenerators B B' and hearth C. The end walls D D of this open-hearth furnace are made thicker or more extended than usual, 40 and in the flues in these walls at each end I provide one or more reducing retorts E E'. As in my former patent, each retort has at its outer end a muffle door, while its inner end, which is preferably closed with a suitable 45 gate K, opens directly onto the melting hearth C. There is also a gas outlet F which may, however, be used for a feed opening. Instead of arranging these retorts horizontally, as in my aforesaid patent, I now arrange them at 50 an angle, as shown, with their inner or discharge ends lower than their outer ends

which are adapted to be closed by the muffle doors.

With a furnace thus constructed, I carry out my improved process of treating fine 55 and pulverized ore for the production of ingots or pig metal, in the following manner: The fine and pulverized ore which is to be treated has added to it a suitable amount of carbon, preferably more than what would be 60 theoretically required to produce a sponge, and there may also be added a small quantity of oxide of manganese and a flux such as lime and any other materials which may be required to produce any special class of 65 metal. I take scrap in a finely divided state, such as borings, turnings, &c., and mix a suitable quantity of that with the ore, as it will facilitate reduction, and improve the product. I then by preference thoroughly mix 70 with the ore, carbon, &c., sufficient liquid, such as water, tar or pitch, to form a stiff plastic mass or mortar, whereby the carbon and manganese and fine scrap if used, will be held in close contact with the ore, and 75 moreover light particles of the ore which would escape if the materials were handled in a dry state will be saved. When the mass has been thoroughly mixed, it can be charged into the retorts at one end of the furnace, the 80 gates K being preferably closed for the time being. When the retorts have been charged, the doors at their outer ends are of course closed. Meantime a bath of scrap or other suitable material which may have been previously heated to near the melting point in 85 one of the retorts, should be thrown onto the hearth C, so that when the flame from the generator is thrown onto the hearth, this material will melt into a suitable bath and the 90 heat from gases passing over the hearth will heat the retorts containing the mixture of pulverized ore and other materials before referred to. When the contents of these retorts on the outgoing side of the furnace have 95 been partially reduced, the gate K may, if desired, be opened to allow the gas to play directly onto the contents which will be quickly brought to a molten state, and owing to the inclined position of the retorts, the molten 100 metal will flow down onto the melting hearth where the action is continued and the molten

metal subjected to the action of the gases for a suitable length of time to complete the melting or reduction. It is then tapped off and cast into ingots, or into pig metal, according to the character of the metal. Meantime the retorts on the opposite side of the hearth have been charged with the pulverized ore and materials combined therewith, so that when the valves in the regenerators are reversed, the contents of those retorts will in turn be melted and flow down onto the hearth.

I claim as my invention—

The mode herein described of treating pulverized ore for the manufacture of iron or

steel, consisting in mixing the ore with finely divided scrap and carbon and subjecting the mixture to heat in a retort and then transferring it to an open hearth, where it is subjected to a further reducing action, all substantially as described.

In testimony whereof I have signed my name to this specification in the presence of two subscribing witnesses.

MICHAEL R. CONLEY.

Witnesses:

EDITH J. GRISWOLD,  
HUBERT HOWSON.